

# UNITED STATES PATENT OFFICE.

ALBERT LANG, OF KARLSRUHE, GERMANY.

## PROCESS FOR THE TREATMENT OF THE SURFACES OF ARTICLES OF ALUMINUM.

1,077,480.

Specification of Letters Patent.

Patented Nov. 4, 1913.

No Drawing.

Application filed February 6, 1907. Serial No. 353,109.

*To all whom it may concern:*

Be it known that I, ALBERT LANG, a subject of the Grand Duke of Baden, Germany, residing at Karlsruhe, in Baden, Germany, 5 have invented a certain new and useful Process for the Treatment of the Surfaces of Articles of Aluminum, of which the following is a specification.

The employment of aluminum for cooking vessels, cartridge cases and for many other useful articles has been found to possess many disadvantages on account of the low melting point of the metal and the fact that it is not hard enough for various purposes, while, however, the low specific gravity would have been of great value. Again the formation on the metal of a layer or coating of oxid for example which would not be easily attacked has been considered impracticable hitherto, on account of the weak affinity of aluminum for acids and alkalies; consequently manufacturers have satisfied themselves with the use of a coating of lacquer or of carbon, or with the 25 application to the aluminum of layers of other metals either as a covering or as intermediate insertions, but these expedients were not satisfactory for various reasons. It has been proposed to color the layers of carbon 30 deposited on the aluminum surface with metallic coloring matters, but of course this coloring is only incorporated with the external covering layers, and is not therefore firmly applied to the metal.

According to the present invention it is possible to form an oxidized coating or layer on the aluminum, this layer having good fire-resisting properties while it is permanent and can if desired be colored or 40 enameled; the layer of color does not rest loosely on the material but becomes permanently bound with the oxidized layer. The oxidized layer may be produced either on the finished article or on the raw material.

45 The oxidation of the surface may be effected by the use of alkali, hydrochloric acid, or metallic chlorids in solution which latter

at the same time produce a colored deposit. Such metallic chlorids may for instance be any of the chlorids of iron or copper. The 50 aluminum object or sheet is dipped in the solution of alkali, hydrochloric acid or the like, or is brushed over with this solution, and the article is subsequently heated to a red heat or incandescence, whereupon, if 55 hydrochloric acid or a chlorid has been used, the chlorin is driven off leaving a hydrate of aluminum, which latter is reduced to the oxid, (alumina), on further heating.

In oxidation as above described by means 60 of metallic salts, such as the chlorids of copper and iron, a colored deposit is produced which may conveniently form the basis for the coloring of the metal; iron gives a gray coloration, copper a black. A coating of 65 enamel may now be applied.

Anilin compounds may be used as coloring agents which become colored by oxidation, or anilin colors may be used which will form compounds of alumina with the 70 oxid layer.

Having thus described my invention I declare what I claim is:

1. The herein described method of treating the surface of aluminum which consists 75 in coating the surface with an oxidizing agent and then subjecting the coated aluminum surface to the action of heat.

2. The herein described method of treating the surface of aluminum which consists 80 in coating the surface with a metallic oxidizing salt and then subjecting the coated aluminum surface to the action of heat.

3. The herein described method of treating the surface of aluminum which consists 85 in coating the surface with a metallic chlorid and then subjecting the coated aluminum surface to the action of heat.

In witness whereof I have hereunto set my hand in presence of two witnesses.

ALBERT LANG.

Witnesses:

SIEGFRIED HAUSER,  
M. L. BRITTAINE.